



US006297067B1

(12) **United States Patent**  
Hattori

(10) **Patent No.:** US 6,297,067 B1  
(45) **Date of Patent:** Oct. 2, 2001

(54) **MANUFACTURE OF FIELD EMISSION ELEMENTS**

(75) Inventor: **Atsuo Hattori**, Hamamatsu (JP)

(73) Assignee: **Yamaha Corporation** (JP)

(\*) Notice: Subject to any disclaimer, the term of this patent is extended or adjusted under 35 U.S.C. 154(b) by 0 days.

(21) Appl. No.: **09/412,925**

(22) Filed: **Oct. 5, 1999**

(30) **Foreign Application Priority Data**

Oct. 7, 1998 (JP) ..... 10-285661

(51) **Int. Cl. 7** ..... **H01L 21/00**

(52) **U.S. Cl.** ..... **438/20**

(58) **Field of Search** ..... 438/20; 445/46,  
445/51

(56) **References Cited**

U.S. PATENT DOCUMENTS

5,599,749 \* 2/1997 Hattori .

\* cited by examiner

*Primary Examiner*—Charles Bowers

*Assistant Examiner*—Evan Pert

(74) *Attorney, Agent, or Firm*—Ostrolenk, Faber, Gerb & Soffen, LLP

(57) **ABSTRACT**

A gate film made of conductive material is formed on a substrate, and a resist pattern having an opening with a predetermined shape is formed on the gate film. The resist pattern is reflowed to make the opening have a tapered shape. By using the resist pattern having the taper shaped opening, the gate film and substrate are anisotropically etched to form a taper shaped opening through the gate film and in the substrate to some depth. After the left resist pattern is etched and removed, the first sacrificial film is formed covering the gate film and substrate with the opening to thereby form an emitter film of conductive material on the first sacrificial film. Unnecessary portions are etched and removed to expose the emitter and gate film and complete a field emission element.

**25 Claims, 28 Drawing Sheets**



**FIG. 1A****FIG. 1B****FIG. 1C**

**FIG. 1D****FIG. 1E****FIG. 1F**

**FIG. 1G****FIG. 1H****FIG. 1I**

**FIG. 1J****FIG. 1K****FIG. 1L**

**FIG.2A****FIG.2B****FIG.2C**

**FIG.2D****FIG.2E****FIG.2F**

19 a

**FIG.3A****FIG.3B****FIG.3C**

**FIG.4**

**FIG. 5A****FIG. 5B****FIG. 5C**

**FIG. 5D****FIG. 5E****FIG. 5F**

**FIG. 5G****FIG. 5H**

**FIG. 6A****FIG. 6B**

**FIG.7A****FIG.7B****FIG.7C**

**FIG. 7D****FIG. 7E****FIG. 7F**

**FIG.7G****FIG.7H****FIG.7I**

**FIG.7J****FIG.7K****FIG.7L**

**FIG. 8A****FIG. 8B****FIG. 8C**

**FIG.8D****FIG.8E****FIG.8F**

**FIG. 9A****FIG. 9B****FIG. 9C**

**FIG. 10**

**FIG. 11A****FIG. 11B****FIG. 11C**

**FIG.11D****FIG.11E****FIG.11F**

**FIG. 11G****FIG. 11H**

**FIG. 12A****FIG. 12B**

**FIG. 13A****FIG. 13B****FIG. 13C**

**FIG. 14**

FIG. 15



**FIG. 16**

## MANUFACTURE OF FIELD EMISSION ELEMENTS

This application is based on Japanese patent application No. 10-285661 filed on Oct. 7, 1998, the entire contents of which are incorporated herein by reference as non-essential subject matter.

### BACKGROUND OF THE INVENTION

#### a) Field of the Invention

The present invention relates to a field emission element, and more particularly to manufacturing technologies for a field emission element having a field emission cathode from the tip of which electrons are emitted.

#### b) Description of the Related Art

A field emission element emits electrons from a sharp tip of an emitter (electron emission cathode) by utilizing electric field concentration. For example, a flat panel display can be structured by using a field emitter array (FEA) having a number of emitters disposed on the array. Each emitter controls the luminance of a corresponding pixel of the display.

In order to apply an electric field to the emitter tip of a field emission element and emit electrons therefrom, the gate electrode biased to a positive potential relative to the emitter (cathode) is disposed near the emitter electrode.

An increase in an emission current from the emitter (i.e., a lowered threshold voltage between the gate and emitter), a high speed drive, and the like are requisites for a field emission element. In order to provide these requisites, it is necessary to devise the structure and shape of a field emission element. It is also necessary to devise a manufacture method in order to manufacture such a field emission element stably and reliably.

A low threshold voltage between the gate and emitter can be achieved by making the distance between the emitter and gate electrode surfaces as gate hole of a gate electrode 100 has a rectangular cross section. There is a danger of a short circuit between the gate and emitter electrodes if a distance between the surface of the emitter electrode 110 and the upper edge of the gate electrode 100 is made short. From this reason, the gate electrode 100 cannot be disposed too near the emitter electrode 110.

If a thickness  $t$  of the gate electrode 100 is made large, an electric field at the tip of the emitter electrode 110 becomes high so that the threshold voltage between the gate and emitter can be lowered without reducing an emission current. In other words, a larger emission current can be obtained without raising a voltage between the gate and emitter. Further, if the thickness  $t$  of the gate electrode 100 is made large, the wiring resistance of the gate electrode 100 becomes low so that a high speed drive becomes possible. However, if the thickness  $t$  of the gate electrode 100 having a rectangular cross section of the gate hole such as shown in FIG. 16 is made large, the danger of the short circuit at the upper edge of the gate electrode 100 increases. In order to avoid this, it is necessary to set a longer distance between the tip surface of the emitter electrode 110 and the surface of the gate electrode 100 by reducing the thickness  $t$ . It is therefore difficult to lower the threshold voltage.

Another requisite for a field emission element is a sharp tip of the emitter electrode 110. Namely, if an apex angle of the tip of the emitter electrode 110 is made small, the electric field at the tip of the emitter electrode 110 becomes high. It is therefore possible to lower a threshold voltage between

the gate and emitter without reducing an emission current, and hence obtain a large emission current without raising a voltage between the gate and emitter. From this reason, it is an important issue to adopt a manufacture method capable of easily sharpening the tip of an emitter electrode 110 having a desired shape.

### SUMMARY OF THE INVENTION

It is an object of the present invention to provide a manufacture method for a field emission element having a structure capable of increasing an emission current from the emitter (i.e., lowering a threshold voltage between the gate and emitter) and executing a high speed drive.

It is another object of the invention to provide a manufacture method for a field emission element having a structure capable of disposing the emitter and gate electrodes as near as possible.

It is another object of the invention to provide a manufacture method for a field emission element capably of sharpening the tip of the emitter electrodes to a large extent.

According to one aspect of the present invention, there is provided a method of manufacturing a field emission element, comprising the steps of: (a) forming a surface layer including a gate film made of a conductive material on a substrate; (b) forming a resist pattern on the surface layer by photolithography, the resist pattern having an opening with a predetermined shape; (c) reflowing the resist pattern to make the opening have an inner diameter gradually reducing toward the substrate; (d) anisotropically etching the gate film by using the reflowed resist pattern as a mask to form an opening through the gate film, the opening having an inner diameter reducing gradually toward the substrate; (e) forming a first sacrificial film covering the gate film having the opening; (f) forming an emitter film made of a conductive material on the first sacrificial film; and (g) removing a portion or a whole of the substrate and a portion of the first sacrificial film to expose the emitter film and the gate film.

According to another aspect of the present invention, there is provided a method of manufacturing a field emission element, comprising the steps of: (a) forming a surface layer including a gate film made of a conductive material on a substrate; (b) forming a low melting point film on the surface layer by photolithography, the low melting point film having a melting point lower than a melting point of the surface layer and an opening with a predetermined shape; (c) reflowing the low melting point film to make the opening have an inner diameter gradually reducing toward the substrate; (d) anisotropically etching the gate film by using the reflowed low melting point film as a mask to form an opening through the gate film, the opening having an inner diameter reducing gradually toward the substrate; (e) forming a first sacrificial film covering the gate film having the opening and/or the low melting point film; (f) forming an emitter film made of a conductive material on the first sacrificial film; and (g) removing a portion or a whole of the substrate and a portion of the first sacrificial film to expose the emitter film and the gate film.

The opening is formed through the gate film, the opening having an inner diameter gradually reducing toward the substrate. This opening allows the surfaces of the gate and emitter electrodes to become near each other in a broad area.

Since such a gently tapered opening is formed by reflowing the resist pattern or low melting point film, the very gentle curve of the opening can be formed with good reproducibility.

By shortening the distance between the surfaces of the emitter and gate electrodes as much as possible without any

danger of a short circuit, a low threshold voltage can be obtained. Furthermore, if the thickness of the gate electrode is made large, an electric field at the tip of the emitter electrode can be made strong so that the threshold voltage between the gate and emitter electrodes can be lowered without reducing the emission current. In other words, a large emission current can be obtained without raising the voltage between the gate and emitter electrodes. If the gate electrode is made thick, the gate wiring resistance lowers so that a high speed drive becomes possible.

If the etching conditions are selected, the shape of the tip of the emitter electrode can be controlled and the tip can be made sharp. Namely, by making small the apex angle of the tip of the emitter electrode, the electric field at the tip can be made strong so that the threshold voltage between the gate and emitter electrodes can be lowered without reducing the emission current, and that a large emission current can be obtained without raising the voltage between the gate and emitter electrodes.

Since the tip of the emitter electrode can be made sharp and the skirt thereof can be made gentle, the process of filling emitter material becomes easy.

#### BRIEF DESCRIPTION OF THE DRAWINGS

FIGS. 1A to 1L are cross sectional views of a substrate illustrating the manufacture processes for a two-electrode field emission element according to a first embodiment of the invention.

FIGS. 2A to 2F are cross sectional views of a substrate illustrating the manufacture processes for a field emission element (two-electrode element) according to a second embodiment of the invention.

FIGS. 3A to 3C are cross sectional views of the substrates of field emission elements according to a modification of the first embodiment.

FIG. 4 is a cross sectional view of the substrate of a field emission element according to a modification of the second embodiment.

FIGS. 5A to 5H are cross sectional views of a substrate illustrating the manufacture processes for a field emission element according to a third embodiment of the invention.

FIGS. 6A and 6B are cross sectional views of the substrates of field emission elements according to a modification of the third embodiment.

FIGS. 7A to 7L are cross sectional views of a substrate illustrating the manufacturing processes for a field emission element according to a fourth embodiment of the invention.

FIGS. 8A to 8F are cross sectional views of a substrate illustrating the manufacture processes for a field emission element according to a fifth embodiment of the invention.

FIGS. 9A to 9C are cross sectional views of the substrates of field emission elements according to a modification of the fourth embodiment.

FIG. 10 is a cross sectional view of the substrates of a field emission element according to a modification of the fourth embodiment.

FIGS. 11A to 11H are cross sectional views of a substrate illustrating the manufacturing processes for a field emission element according to a sixth embodiment of the invention.

FIGS. 12A and 12B are cross sectional views of the substrates of field emission elements according to a modification of the sixth embodiment.

FIGS. 13A to 13C are cross sectional views of substrates illustrating a taper shape changed with a difference of an etching rate between resist and a gate electrode film.

FIG. 14 is a perspective view of a field emission element according to an embodiment of the invention.

FIG. 15 is a cross sectional view of a flat panel display using field emission elements.

FIG. 16 is a cross sectional view of a field emission element.

#### DETAILED DESCRIPTION OF THE PREFERRED EMBODIMENTS

FIGS. 1A to 1L are cross sectional views of a substrate illustrating the manufacture processes for a field emission element according to the first embodiment of the invention. In the following, the manufacture processes for a two-electrode element having an emitter (field emission cathode) and a gate will be described. The two-electrode element has two electrodes, an emitter electrode for emitting electrons and a gate electrode for controlling an electric field.

Referring to FIG. 1A, a gate electrode film 11 made of first conductive material is formed on a single layer substrate 10 made of, for example, glass, quartz or the like or on a substrate 10 made of a lamination of an Si layer and a silicon oxide film formed thereon. The first material of the gate electrode film 11 is silicon doped with P (phosphorous) or B (boron) and deposited to a thickness of about 1  $\mu\text{m}$ .

For example, the gate electrode film 11 made of silicon is formed under the conditions of a source gas of  $\text{SiH}_4$  diluted with He and a substrate temperature of 625° C. In order to lower the resistance value of the gate electrode film 11, P or B ions are diffused or implanted into the gate electrode film 11.

As shown in FIG. 1B, resist material is coated on the gate electrode film 11 and etched through photolithography to form a resist pattern 12 having an opening 13 of about 0.45  $\mu\text{m}$  in diameter. The opening 13 is cylindrical having a rectangular cross section and a circle plan view having the diameter of about 0.45  $\mu\text{m}$ . This resist pattern is formed by the following processes.

For example, photoresist material of the resist pattern 12 is i-line (365 nm) resist THMR-iP3100 manufactured by Tokyo Ohka Kogyo Co. Ltd. and coated to a thickness of about 0.1  $\mu\text{m}$ . In order to improve the size precision of the pattern, it is preferable to coat AZ-AQUATAR manufactured by Clariant (Japan) K.K. to a thickness of about 0.064  $\mu\text{m}$  on the resist material as an upper coated antireflection film.

The resist is exposed to light by using an i-line stepper NSR2005i11D manufactured by Nikon Corp. and a reticle having a predetermined pattern under the conditions of  $\text{NA}=0.57$  and  $\text{sigma}=0.4$ . Thereafter, the resist is developed for 60 seconds by using NMD-3 (TMAH: tetra methyl ammonium hydroxide) manufactured by Tokyo Ohka Kogyo Co., Ltd., and thereafter rinsed with pure water.

Next, the resist pattern 12 is baked (reflowed), for example, by a hot plate (not shown) at a temperature of 150° C. for about 90 seconds to form a resist pattern 12a having a gentle slope upper corner as shown in FIG. 1C. A recess 13a has a taper shape in cross section having an inter diameter large at the higher level and gradually making small toward a lower level. The resist pattern 12 may be exposed to ultraviolet rays before it is reflowed. When it is exposed to ultraviolet rays, the temperature for reflowing the resist pattern 12 can be lowered by about 10° C. to 20° C.

Next, by using the reflowed resist pattern 12a as a mask, the gate electrode film 11 made of the first conductive material is etched to form a recess (gate hole) 13b having a gentle tapered side wall. The recess 13b has a gently curved

cross section gradually making its inner diameter small toward the substrate **10** (lower portion).

This etching is an over-etch to etch the substrate **10** by about  $0.1 \mu\text{m}$  in depth from the surface of the substrate **10** to form a substrate **10a** having a recess. This depth influences the length of an emitter electrode to be later formed. The diameter of the recess **13b** of the gate electrode film **11a** is about  $0.5 \mu\text{m}$  at the bottom and about  $1.5 \mu\text{m}$  at the upper level, and the depth is about  $1 \mu\text{m}$ .

For example, this etching is performed by using a reactive ion etching (RIE) system under the conditions of an etching gas of  $\text{CO}_2+\text{CHF}_3+\text{Ar}$  and a reaction chamber pressure of 125 mTorr. Etching rate of the gate electrode film **11** is about  $1.2 \mu\text{m}/\text{min}$  and etching rate of the resist pattern **12a** is about  $0.8 \mu\text{m}/\text{min}$ .

Next, as shown in FIG. 1E, the left resist **12b** is removed. For example, in order to remove the resist **12b**,  $\text{H}_2\text{SO}_4+\text{H}_2\text{O}_2$  heated to  $140^\circ\text{C}$ . is used. Ashing by oxygen plasma or remover such as N-methyl-2-pyrrolidone may also be used.

Next as shown in FIG. 1F, a first sacrificial film (insulating film) **14** of silicon oxide is isotropically deposited on the whole substrate surface to a thickness of  $0.3 \mu\text{m}$  by atmospheric pressure chemical vapor deposition (CVD). For example, the first sacrificial film **14** is formed under the conditions of a source gas of  $\text{O}_3$  and TEOS and a substrate temperature of  $400^\circ\text{C}$ . Under these conditions, the first sacrificial film **14** is deposited inheriting (conformal to) the side wall surface shape of the recess **13b**.

Next as shown in FIG. 1G, a first emitter electrode film **15** of second conductive material such as  $\text{TiN}_x$  is isotropically deposited on the first sacrificial film **14** to a thickness of  $0.05 \mu\text{m}$  by reactive sputtering. This reactive sputtering is performed by using a DC sputtering system and Ti as a target while a gas of  $\text{N}_2$  and Ar is introduced. The first emitter electrode film **15** is therefore formed inheriting (conformal to) the surface shape of the first sacrificial film **14**.

The emitter electrode **15** has a two-stage shape. The first stage depends upon the tapered side wall of the gate electrode **11a** and the second stage depends upon the upper corner of the gate electrode **11**.

Next, as shown in FIG. 1H, a second emitter electrode film **16** made of third conductive material is deposited on the first emitter electrode film **15** to a thickness of  $0.2 \mu\text{m}$ , the second electrode film **16** serving as a blanket film. For example, the third conductive material is W and is deposited by CVD under the condition of a gas of  $\text{WF}_6+\text{H}_2+\text{N}_2+\text{Ar}$ , a pressure of 80 Torr and a temperature of  $450^\circ\text{C}$ .

Next, as shown in FIG. 1I, the second emitter electrode film **16** is etched back by  $0.2 \mu\text{m}$  in thickness to leave only a blanket film **16a**. The blanket film **16a** fills a recess of the first emitter electrode film **15**. The etch-back is performed by using an RIE system under the conditions of an etching gas of  $\text{SF}_6+\text{Ar}+\text{He}$  and a reaction chamber pressure of 280 mTorr.

It is known that in order to sufficiently stabilize an emission current from a field emission cathode (emitter), a resistor layer is connected serially to the emitter. As shown in FIG. 1J, therefore, a resistor layer **17** of silicon is deposited to a thickness of about  $0.2 \mu\text{m}$  on the first emitter electrode **15** and blanket film **16a** by sputtering.

The silicon film (resistor layer) **17** is sputtered by using a DC sputtering system and Si as a target while Ar gas is introduced. Instead of an Ar gas, a gas of  $\text{N}_2+\text{Ar}$ ,  $\text{O}_2+\text{Ar}$ , or  $\text{N}_2+\text{O}_2+\text{Ar}$  may be used with reactive sputtering to form a

resistor layer **17** of  $\text{SiN}_x$ ,  $\text{SiO}_x$  or  $\text{SiO}_x\text{N}_y$  having an increased resistance value. Instead of sputtering, vapor deposition or plasma CVD may also be used for forming the resistor layer.

Next as shown in FIG. 1K, an emitter wiring layer **18** made of fourth conductive material such as Al is deposited on the resistor layer **17** to a thickness of about  $0.5 \mu\text{m}$  by sputtering. For example, this sputtering is performed by using a DC sputtering system and Al as a target while Ar gas is introduced.

Lastly as shown in FIG. 1L, the substrate **10a** and a portion of the first sacrificial film **14** are etched and removed to expose the gate electrode **11a** and first emitter electrode **15** to complete a two-electrode element. For etching Si such as Si substrate,  $\text{HF}+\text{HNO}_3+\text{CH}_3\text{COOH}$  is used, and for etching a silicon oxide film or the like,  $\text{HF}+\text{NH}_4\text{F}$  is used.

The emitter electrode **15** having a two-stage shape has a sharp tip and can easily emit electrons. Since the skirt portion of the emitter electrode can be made to have a gentle slope, a process of filing emitter material becomes easy.

According to the first embodiment, similar to the emitter electrode the gate electrode **11a** has a tapered side wall so that a distance between the gate electrode **11a** and emitter electrode **15** can be made short. It is therefore possible to raise an electric field intensity at the tip of the emitter electrode and manufacture a field emission element having a low threshold voltage.

Also according to the first embodiment, the position in height (position in the vertical direction) of the emitter electrode is determined by the over-etch depth of the substrate **10** shown in FIG. 1D and the thickness of the first sacrificial film **14** shown in FIG. 1F. A distance between the emitter electrode **15** and gate electrode **11a** is determined by the thickness of the first sacrificial film **14**. The shape of the emitter electrode **15** and the tapered shape of the gate hole of the gate electrode **11a** are determined by the reflow process shown in FIG. 1C and the etching process shown in FIG. 1D. By properly setting these parameters, the position in height of the emitter electrode, the shapes of the gate and emitter electrodes, a distance between the emitter and gate electrodes and the like can be controlled with good reproducibility.

It has been found from the experiments made by the inventor that a slope angle  $\theta_r$  (an angle of a wall in the recess **13a** relative to the substrate surface which angle is smaller than  $90^\circ$ ) of the taper shaped recess **13a** becomes smaller as the resist reflow temperature is set higher during the reflow process shown in FIG. 1C. This tendency becomes stronger the larger the diameter of the recess **13a**. Namely, as the diameter becomes smaller, it becomes harder for the resist to soften. The thickness of the resist also influences the slope angle. If the resist is baked at the temperature of  $180^\circ\text{C}$ ., the resist flows completely. In the range from  $100$  to  $140^\circ\text{C}$ ., the slope angle is hard to be changed. It is therefore preferable to set the reflow temperature to a range higher than  $140^\circ\text{C}$ . and lower than  $180^\circ\text{C}$ ., or more preferably a range from about  $150^\circ\text{C}$ . to  $160^\circ\text{C}$ . The temperature range may change depending upon the resist material.

Experiment results of the etching process shown in FIG. 1D of this embodiment will be described with reference to FIGS. 13A to 13C. The tapered shape of the recess **13b** is not only determined by the shape of the resist but also can be controlled by a selection ratio (etching rate ratio) during the etching process shown in FIG. 1D. FIGS. 13A to 13D show the tapered shapes obtained by the etching processes with different selection ratios made by the inventor.  $R_r$  represents

an etching rate of the resist **12b** and  $R_g$  represents an etching rate of the gate electrode film **11a**.

The tapered shape shown in FIG. 13A was formed by an etching process under the condition of  $R_r < R_g$ . In this case, since a retraction (thickness reduction) of the resist during the etching process is small, the slope angle  $\theta_g$  of the gate hole cross section of the gate electrode **11a** is large.

The tapered shape shown in FIG. 13B was formed by an etching process under the condition of  $R_r = R_g$  (selection ratio=1). In this case, as compared to the tapered shape shown in FIG. 13A, the slope angle  $\theta_g$  of the gate hole cross section of the gate electrode **11a** becomes smaller. The tapered shape shown in FIG. 13C was formed by an etching process under the condition of  $R_r > R_g$ . In this case, the slope angle  $\theta_g$  of the gate hole cross section of the gate electrode **11a** becomes much smaller and the thickness of the left resist film **12b** reduces. The preferable condition is as follows to obtain a preferable tapered shape.

$$20^\circ < \theta_g < 80^\circ$$

$$0.2 < (R_r/R_g) < 5.0$$

$$0.5 < (R_r/R_g) < 2.0 \text{ (more preferable)}$$

It is preferable that a melting point of the material of the gate electrode **11** and substrate **10** to be etched is higher than the reflow temperature of the resist. The material of the gate electrode film **11** satisfying this condition may be semiconductor such as polysilicon, metal such as W and Al and silicide such as  $WSi_x$  and  $TiSi_x$ . A gate electrode film **11** whose upper and lower surfaces are laminated by an insulating film such as a silicon oxide film and a silicon nitride film or an antireflection film such as  $TiN_x$  and  $TiO_xN_y$  may be etched to form a tapered shape. The substrate **10** may be made of glass, quartz, silicon laminated with a silicon oxide film, aluminum laminated with an anodized aluminum film or the like.

FIGS. 2A to 2F are cross sectional views of a substrate illustrating the manufacture processes for a field emission element according to the second embodiment of the invention. Also in this embodiment, a two-electrode element having an emitter and gate is manufactured.

Referring to FIG. 2A, a gate electrode film **21** made of first conductive material is formed on a single layer substrate **20** made of, for example, glass, quartz or the like or on a substrate **10** made of a lamination of an Si layer and a silicon oxide film formed thereon. The first material of the gate electrode film **21** is silicon doped with P (phosphorous) or B (boron) and deposited to a thickness of about  $0.5 \mu m$ .

For example, the gate electrode film **21** made of silicon is formed under the conditions of a source gas of  $SiH_4$  diluted with  $H_e$ , a substrate temperature of  $625^\circ C$ , and a reaction chamber pressure of 30 Pa. In order to lower the resistance value of the gate electrode film **21**, P or B ions are diffused or implanted into the gate electrode film **21**.

In order to improve the dielectric breakdown voltage between the gate and emitter electrodes and lower the capacitance therebetween, a first sacrificial film (insulating film) **22** of silicon nitride is deposited on the whole substrate surface to a thickness of  $0.5 \mu m$  by low pressure CVD. For example, the low pressure CVD is performed under the conditions of a gas of  $NH_3$  and  $SiH_2Cl_2$ , a substrate temperature of  $750^\circ C$  and a temperature of 60 Pa. The silicon nitride film may be formed by plasma CVD or reactive sputtering.

In order to improve a size precision of a gate hole to be later formed, an antireflection film of  $SiN_x$ ,  $SiO_x$  and  $TiN_x$  may be used as the first sacrificial film **22**.

Instead of silicon nitride, the first sacrificial film **22** may be made of getter material such as Ti, Ta and zirconium in order to improve the vacuum degree near emitter elements of a field emission emitter array (flat panel display shown in FIG. 15) and suppress the attachment of molecules to the surface of the emitter electrode.

As shown in FIG. 2B, resist material is coated on the first sacrificial film **22** and etched through photolithography to form a resist pattern **24** having an opening **23** of about  $0.45 \mu m$  in diameter at the surface level, by processes similar to those described with FIG. 1B.

Next, the resist pattern **24** is baked (reflowed), for example, by a hot plate (not shown) at a temperature of  $150^\circ C$  for about 90 seconds to form a resist pattern **24a** having a recess **23a** with a gentle slope upper corner as shown in FIG. 1C. The recess **23a** has a gentle taper shape in cross section having an inter diameter large at the higher level and gradually making small toward a lower level.

Next, by using the reflowed resist pattern **24a** as a mask, the gate electrode film **21** made of the first conductive material and the first sacrificial film **22** are etched to form a recess (gate hole) **23b** having a gentle tapered side wall as shown in FIG. 2D. This etching is an over-etch to etch the substrate **20** by about  $0.1 \mu m$  in depth from the surface of the substrate **20** and form a substrate **20a** having a recess. The depth of this recess influences the length of an emitter electrode to be later formed. The diameter of the recess **23b** of the gate electrode film **21a** is about  $0.5 \mu m$  at the bottom and about  $0.7 \mu m$  at the upper level, and the depth is about  $0.5 \mu m$ .

For example, this etching is performed by using a magnetron RIE system under the conditions of an etching gas of  $CO_2+CHF_3+Ar$  and a reaction chamber pressure of 125 mTorr. Etching rates of the gate electrode film **21**, the first sacrificial film **22** and the resist pattern **24a** are about  $1.2 \mu m/min$ ,  $1.2 \mu m/min$  and  $0.8 \mu m/min$ , respectively.

Next, by using processes similar to those described with reference to FIGS. 1E to 1G of the first embodiment, the left resist **24b** is removed, and thereafter as shown in FIG. 2E, a second sacrificial film (insulating film) **25** of silicon oxide is deposited on the whole substrate surface to a thickness of  $0.15 \mu m$  by atmospheric pressure CVD, and a first emitter electrode film **26** of second conductive material such as  $TiN_x$  is deposited on the second sacrificial film **25** to a thickness of  $0.05 \mu m$  by reactive sputtering.

Next, after performing processes similar to those described with reference to FIGS. 1H to 1K of the first embodiment, a blanket film **27a**, a resistor film **28** and an emitter wiring layer **29** are sequentially laminated as shown in FIG. 2F. Lastly, similar to the process shown in FIG. 1L, the substrate **20a** and a portion of the second sacrificial film **25** are etched and removed to expose the gate electrode **21a** and emitter electrode **26** to complete a two-electrode element.

According to the second embodiment, by using the first and second sacrificial films **22a** and **25a** made of insulating material are used to make the gate electrode **21a** thinner than that of the first embodiment. Therefore, the capacitance between the gate and emitter electrodes becomes small and the dielectric breakdown voltage between the gate and emitter electrodes can be improved.

FIGS. 3A to 3C illustrate methods of reinforcing the emitter electrode with a support substrate according to a modification of the first embodiment.

With the method shown in FIG. 3A, a recess on the surface of the emitter electrode of the element subjected to the processes shown in FIGS. 1A to 1G of the first embodiment

ment is filled with a planarizing layer **19a** made of, for example, spin-on-glass (SOG). Thereafter, the surface of the planarizing film **19a** is planarized by chemical mechanical polishing (CMP) or whole surface etching. Then, a support substrate **19b** is adhered to the planarizing film **19a** by electrostatic adhesion or by using adhesive.

Thereafter, the unnecessary portions such as substrate **10a** are etched and removed by a process similar to the etching process shown in FIG. 1L, to expose the gate electrode **11a** and emitter electrode **15** as shown in FIG. 3A and complete a two-electrode element.

Also with the method shown in FIG. 3B, the emitter electrode **15** of the element subjected to the processes shown in FIGS. 1A to 1G of the first embodiment is adhered to a support substrate **19b** by using adhesive **19c** such as low melting point glass.

Thereafter, the unnecessary portions such as substrate **10a** are etched and removed by a process similar to the etching process shown in FIG. 1L, to expose the gate electrode **11a** and emitter electrode **15** as shown in FIG. 3B and complete a two-electrode element.

With the method shown in FIG. 3C, a recess on the surface of the emitter electrode of the element subjected to the processes shown in FIGS. 1A to 1G of the first embodiment is filled with a planarizing layer **19a** made of, for example, SOG. Thereafter, the surface of the planarizing film **19a** is planarized by CMP. Then, a support substrate **19b** is adhered to the planarizing film **19a** and emitter electrode **15** by using adhesive **19c** such as low melting point glass.

Thereafter, the unnecessary portions such as substrate **10a** are etched and removed by a process similar to the etching process shown in FIG. 1L, to expose the gate electrode **11a** and emitter electrode **15** as shown in FIG. 3C and complete a two-electrode element.

FIG. 4 illustrates a method of reinforcing the emitter electrode with a support substrate according to a modification of the second embodiment.

With the method shown in FIG. 4, a recess on the surface of the emitter electrode **26** of the element subjected to the processes shown in FIGS. 2A to 2E of the second embodiment is filled with a planarizing layer **27f** made of, for example, SOG. Thereafter, the surface of the planarizing film **27f** is planarized by CMP or whole surface etching. Then, a support substrate **27s** is adhered to the emitter electrode **26** and planarizing film **27f** by using adhesive **27g** such as low melting glass.

Thereafter, the unnecessary portions such as substrate **20a** are etched and removed by a process similar to the etching process shown in FIG. 2F, to expose the gate electrode **21a** and emitter electrode **26** as shown in FIG. 4 and complete a two-electrode element. FIGS. 5A to 5H are cross sectional views of a substrate illustrating the manufacture processes for a field emission element (three-electrode element) according to the third embodiment of the invention. The three-electrode element of the third embodiment has three electrodes, an emitter electrode, a gate electrode and an anode electrode.

Referring to FIG. 5A, a substrate **30** is formed by depositing an anode electrode film **30b** made of first conductive material to a thickness of  $0.1 \mu\text{m}$  by low pressure CVD, on either a single layer substrate **30a** made of, for example, glass, quartz or the like or on a substrate **30a** made of a lamination of an Si layer and a silicon oxide film formed thereon, and by forming a first sacrificial film (insulating film) **30c** made of silicon oxide on the anode electrode film **30b** to a thickness of  $0.1 \mu\text{m}$  by atmospheric pressure CVD.

In this case, the first conductive material of the anode electrode **30b** is silicon doped with P or B in order to lower

the resistance value. The anode electrode **30b** is formed under the conditions of a source gas of  $\text{SiH}_4$  diluted with He, a substrate temperature of  $625^\circ \text{C}$ . and a reaction chamber pressure of 30 Pa. The first sacrificial film **30c** is formed under the conditions of a source gas of  $\text{O}_3$  and TEOS, and a substrate temperature of  $400^\circ \text{C}$ .

On the first sacrificial film **30c** of the substrate **30** formed as above, a gate electrode film made of second conductive material is formed. The second conductive material of the gate electrode film **31** is made of silicon doped with P (phosphorous) or B (boron) and deposited to a thickness of about  $0.3 \mu\text{m}$ . For example, this gate electrode film **31** made of silicon is formed by low pressure CVD under the conditions of a source gas of  $\text{SiH}_4$  diluted with He, a substrate temperature of  $625^\circ \text{C}$ . and a reaction chamber pressure of 30 Pa. In order to lower the resistance value of the gate electrode film **31**, P or B ions are diffused or implanted into the gate electrode film **31**.

Further, as shown in FIG. 5A, resist material is coated on the gate electrode film **31** and etched through photolithography to form a resist pattern **32** having an opening **33** of about  $0.45 \mu\text{m}$  in diameter at its surface.

For example, i-line (365 nm) resist THMR-iP3100 manufactured by Tokyo Ohka Kogyo Co. Ltd. is coated to a thickness of about  $0.5 \mu\text{m}$ . In order to improve the size precision of the resist pattern **32**, it is preferable to coat AZ-AQUATAR manufactured by Clariant (Japan) K.K. to a thickness of about  $0.064 \mu\text{m}$  the resist material as a coated antireflection film.

The resist is exposed to light by using an i-line stepper NSR2005i11D manufactured by Nikon Corp. and a reticle having a predetermined pattern under the conditions of  $\text{NA}=0.57$  and  $\text{sigma}=0.4$ . Thereafter, the resist is developed for 60 seconds by using NMD-3 (TMAH: tetra methyl ammonium hydroxide 2.38%) manufactured by Tokyo Ohka Kogyo Co., Ltd., and thereafter rinsed with pure water.

Next, the resist pattern **32** is baked (reflowed), for example, by a hot plate (not shown) at a temperature of  $150^\circ \text{C}$ . for about 90 seconds to form a resist pattern **32a** having a recess **33a** with a gentle slope upper corner as shown in FIG. 5B. The recess **33a** has a taper shape in cross section having an inter diameter large at the higher level and gradually making small toward a lower level.

Next, by using the reflowed resist pattern **32a** as a mask, the gate electrode film **31** made of silicon and first sacrificial film **30c** are etched to form a recess (gate hole) **33b** having a gentle tapered side wall. It is preferable to over-etch the substrate **30** by about  $0.1 \mu\text{m}$  (corresponding to a thickness of the first sacrificial film **30c**) in depth from the surface of the substrate **30** to form a substrate **30** having a recess. The depth of the recess influences the height and length of an emitter electrode to be later formed.

For example, this etching is performed by using a magnetron RIE system under the conditions of an etching gas of  $\text{CO}_2+\text{CHF}_3+\text{Ar}$  and a reaction chamber pressure of 125 mTorr. Etching rates of the gate electrode film **31** and the resist pattern **32a** are about  $1.2 \mu\text{m}/\text{min}$  and  $0.8 \mu\text{m}/\text{min}$ , respectively.

Next, as shown in FIG. 5D, the leftover resist **32b** is removed. For example, in order to remove the resist **32b**,  $\text{H}_2\text{SO}_4+\text{H}_2\text{O}_2$  heated to  $140^\circ \text{C}$ . is used. Shing by oxygen plasma or remover such as N-methyl-2-pyrrolidone may also be used.

Next as shown in FIG. 5E, a second sacrificial film (insulating film) **34** of silicon oxide is isotropically deposited on the whole substrate surface to a thickness of  $0.3 \mu\text{m}$  by atmospheric pressure CVD. For example, the second

sacrificial film **34** is formed under the conditions of a source gas of  $O_3$  and TEOS and a substrate temperature of  $400^\circ C$ . Under these conditions, the second sacrificial film **34** is deposited inheriting (conformal to) the side wall surface shape of the recess **33b**.

Next as shown in FIG. 5F, an emitter electrode film **35** of third conductive material such as  $TiN_x$  is isotropically deposited on the second sacrificial film **34** to a thickness of  $0.05 \mu m$  by reactive sputtering. This reactive sputtering is performed by using a DC sputtering system and Ti as a target while a gas of  $N_2$  and Ar is introduced. The emitter electrode film **35** is therefore formed inheriting (conformal to) the surface shape of the second sacrificial film **34**.

Next, a resist mask (not shown) having a predetermined opening is formed on the whole surface of the emitter electrode film **35** by using ordinary photolithography. A portion of the emitter electrode **35** not used as the cathode is etched and removed through the opening to form a slit opening **36** shown in FIG. 5G. For example, this etching is performed by using a magnetron RIE system under the conditions of a gas of  $Cl_2$  and a reaction chamber pressure of  $125 \text{ mTorr}$ . On the second sacrificial film **34**, emitter electrodes **35a** and **35b** having predetermined patterns as viewed in cross section are therefore left.

Next, via the slit opening **36**, portions of the second and first sacrificial films **34** and **30c** are etched to expose the gate electrode **31a**, emitter electrode **35a** and anode electrode **30b** and complete a three-electrode element as shown in FIG. 5H. For etching the first and second sacrificial films **30c** and **34** of silicon oxide,  $HF+NH_4F$  is used.

The three-electrode element has the emitter electrode as a cathode and the anode electrode **30** as a plate. As a positive potential having a predetermined value is applied to the gate electrode, an electron beam is emitted from the emitter electrode **35a** toward the anode electrode **30b** while being converged.

FIG. 6A shows a three-electrode element modified from a two-electrode element of the second embodiment. The manufacture method and structure of a substrate are the same as the third embodiment shown in FIG. 5A. By using processes similar to those shown in FIGS. 2A to 2E, an Si gate electrode film **21a**, an  $SiN_x$  second sacrificial film **22a**, an  $SiO_2$  third sacrificial film **25** and a  $TiN_x$  emitter electrode **26** are formed on the substrate **30**.

Next, by using a process similar to that shown in FIG. 5G, a resist mask (not shown) having a predetermined opening is formed on the whole surface of the emitter electrode film **26** by using ordinary photolithography. A portion of the emitter electrode **26a** not used as the cathode is etched and removed through the opening to form a slit opening **26c** shown in FIG. 6A. Next, by using a process similar to that shown in FIG. 5H, via the slit opening **26c**, portions of the third and first sacrificial films **25a** and **30c** are etched to expose the gate electrode **21a**, emitter electrode **26a** and anode electrode **30b** and complete a three-electrode element.

FIG. 6B shows another example of a three-electrode element modified from a two-electrode element of the second embodiment. The structure different from that shown in FIG. 6A is that the second sacrificial film **22a** is made of the same material  $SiO_2$  as the material of the first and third sacrificial films **30c** and **25a**.

By using a process similar to that shown in FIG. 5G, a resist mask (not shown) having a predetermined opening is formed on the whole surface of the emitter electrode film **26** by using ordinary photolithography. A portion of the emitter electrode **26** not used as the cathode is etched and removed through the opening to form a slit opening **26c** shown in

FIG. 6B. Next, by using a process similar to that shown in FIG. 5H, via the slit opening **26c**, portions of the third, second and first sacrificial films **25a**, **22a** and **30c** are etched. In this case, since the third, second and first sacrificial films **25a**, **22a** and **30c** are made of the same silicon oxide material, the etching rates are the same. Since the unnecessary portions are removed, the gate electrode **21a**, emitter electrode **26a** and anode electrode **30b** are exposed and a three-electrode element is completed as shown in FIG. 6B.

FIG. 7A to 7L are cross sectional views of a substrate illustrating the manufacture processes for a field emission element according to the fourth embodiment of the invention. In the embodiment, the manufacture processes for a two-electrode element having an emitter (field emission cathode) and a gate will be described.

In the first to third embodiments, a tapered recess is formed by heating a resist film and by using this tapered shape an emitter electrode is formed. In the fourth embodiment to be described hereinafter, instead of the resist film, a reflow film made of low melting material (material having a melting point lower than that of electrode material and other materials of layers laminated on the upper and lower surfaces of each electrode layer) is used to form a tapered recess, and an emitter electrode is formed by using this recess.

Referring to FIG. 7A, a gate electrode film **41** made of first conductive material is formed on a single layer substrate **40** made of, for example, quartz or the like or on a substrate **40** made of a lamination of an  $Si$  layer and a silicon oxide film formed thereon. The first conductive material of the gate electrode film **41** is silicon doped with P (phosphorous) or B (boron) and deposited to a thickness of about  $0.3 \mu m$  by low pressure CVD.

For example, the gate electrode film **41** made of silicon is formed under the conditions of a source gas of  $SiH_4$  diluted with He, a substrate temperature of  $625^\circ C$ . and a reaction chamber pressure of  $30 \text{ Pa}$ . In order to lower the resistance value of the gate electrode film **41**, P or B impurity ions are diffused or implanted into the gate electrode film **41**.

A low melting point film (low temperature reflow film) **42** is formed on the gate electrode film **41**. For example, the low melting point film **42** is made of phosphosilicate glass (PSG) deposited to a thickness of about  $0.5 \mu m$ . Instead of PSG, other low melting glass may be used such as borophosphosilicate glass (BPSG), borosilicate glass (BSG), arsenosilicate glass (AsSG), arsenophosphosilicate glass (AsPSG) and phosphogermanosilicate glass (PGSG), frit glass, covar, solder,  $Si$ — $Ge$ , or low melting point metal. The low melting point film may be a single layer film or a lamination film. If a low melting point film having a lamination structure is used, the material of the uppermost layer thereof is selected to have a lowest melting point.

Next as shown in FIG. 7B, photoresist material is coated on the low melting point film **42** and etched through photolithography to form a resist pattern **43** having an opening **43a** of about  $0.45 \mu m$  in diameter at its surface level. This resist pattern **43** having the opening **43a** is formed by the following processes.

For example, i-line (365 nm) resist THMR-iP3100 manufactured by Tokyo Ohka Kogyo Co. Ltd. is coated to a thickness of about  $0.1 \mu m$  as the material of the resist pattern **43**. In order to improve the size precision of the resist pattern **43**, it is preferable to coat AZ-AQUATAR manufactured by Clariant (Japan) K.K. to a thickness of about  $0.064 \mu m$  on the resist material as a coated antireflection film.

The resist is exposed to light by using an i-line stepper NSR2005i11D manufactured by Nikon Corp. and a reticle

having a predetermined pattern under the conditions of  $NA=0.57$  and  $\sigma=0.4$ . Thereafter, the resist is developed for 60 seconds by using NMD-3 (TMAH: tetra methyl ammonium hydroxide) manufactured by Tokyo Ohka Kogyo Co., Ltd., and thereafter rinsed with pure water.

Next, by using the resist pattern 43 as a mask, the low melting point film 42 is anisotropically etched to form a low melting point film 42a having an opening 42b as shown in FIG. 7C. This opening 42b has a vertical or a generally vertical side wall reaching the gate electrode film 41. For example, this etching is performed by using a magnetron RIE under the conditions of an etching gas of  $CHF_3+CO_2+Ar+He$  and a reaction chamber pressure of 50 mTorr. After the etching, the leftover resist is removed. In order to prevent the resist from being softened during the etching, it is preferable to cool the bottom surface of the substrate 40 with He.

Next, the low melting point film 42a is heated and reflowed to form a low melting point film pattern 42d having a tapered recess 42c with a gentle slope upper corner or shoulder, as shown in FIG. 7D. For example, this reflow process is performed by using a furnace under the conditions of an atmosphere of  $N_2$  and a temperature of 1000° C. for about 30 minutes. Lamp heating or laser heating may also be used. The specific conditions and the like of the reflow process will be detailed with reference to the accompanying drawings after the description of the processes of this embodiment.

Next, by using the reflowed low melting point film pattern 42d as a mask, the gate electrode film 41 made of the first conductive material is etched to form a recess (gate hole) 42e having a gentle tapered side wall, as shown in FIG. 7E and to form a reduced thickness low melting point film pattern 42f. This etching is an over-etch to etch the substrate 40 by about 0.1  $\mu m$  in depth from the surface of the substrate 40 to form a substrate 40a having a recess. The depth of this recess influences the length and height of an emitter electrode to be later formed. The diameter of the recess 42e of the gate electrode film 41a is about 0.51  $\mu m$  at the bottom and about 0.7  $\mu m$  at the upper level, and the depth is about 0.3  $\mu m$ . The depth of this recess influences the length and height of an emitter electrode to be later formed. The diameter of the recess 42e of the gate electrode film 41a is about 0.5  $\mu m$  at the bottom and about 0.7  $\mu m$  at the upper level, and the depth is about 0.3  $\mu m$ .

For example, this etching is performed by using a magnetron RIE system under the conditions of an etching gas of  $CO_2+CHF_3+Ar$  and a reaction chamber pressure of 125 mTorr. Etching rates of the gate electrode film 41 and the low melting point film pattern 42d are about 1.2  $\mu m/min$  and 1.0  $\mu m/min$ , respectively.

Next, as shown in FIG. 7F, a first sacrificial film (insulating film) 44 of silicon oxide is isotropically deposited on the whole substrate surface to a thickness of 0.3  $\mu m$  by atmospheric pressure CVD. For example, the first sacrificial film 44 is formed under the conditions of a source gas of  $O_3$  and TEOS and a substrate temperature of 400° C. Under these conditions, the first sacrificial film 44 is deposited inheriting (conformal to) the side wall surface shape of the recess 42e.

Next as shown in FIG. 7G, a first emitter electrode film 45 of second conductive material such as  $TiN_x$  is isotropically deposited on the first sacrificial film 44 to a thickness of 0.05  $\mu m$  by reactive sputtering. This reactive sputtering is performed by using a DC sputtering system and Ti as a target while a gas of  $N_2+Ar$  is introduced. The first emitter electrode film 45 is therefore formed inheriting (conformal to) the surface shape of the first sacrificial film 44.

Next, as shown in FIG. 7H, a second emitter electrode film 46 made of third conductive material is deposited on the first emitter electrode film 45 to a thickness of 0.2  $\mu m$ , the second electrode film 46 serving as a blanket film. For example, the third conductive material is W and is deposited by CVD under the condition of a gas of  $WF_6+H_2+N_2+Ar$ , a pressure of 80 Torr and a temperature of 450° C.

Next, as shown in FIG. 7I, the second emitter electrode film 46 is etched back by 0.2  $\mu m$  in thickness to leave only a blanket film 46a. The etch-back is performed by using an RIE system under the conditions of an etching gas of  $SF_6+Ar+He$  and a reaction chamber pressure of 280 mTorr.

It is known that in order to sufficiently stabilize an emission current from a field emission cathode (emitter), a resistor layer is connected serially to the emitter. As shown in FIG. 7J, therefore, a resistor layer 47 of silicon is deposited to a thickness of about 0.2  $\mu m$  on the first emitter electrode 45 and blanket film 46a by sputtering.

The resistor layer 47 is sputtered by using a DC sputtering system and Si as a target while Ar gas is introduced. Instead of an Ar gas, a gas of  $N_2+Ar$ ,  $O_2+Ar$ , or  $N_2+O_2+Ar$  may be used with reactive sputtering to form a resistor layer 47 of  $SiN_x$ ,  $SiO_x$  or  $SiO_xN_y$  having an increased resistance value. Instead of sputtering, vapor deposition or plasma CVD may also be used for forming the resistor layer.

Next as shown in FIG. 7K, an emitter wiring layer 48 made of fourth conductive material such as Al is deposited on the resistor layer 47 to a thickness of about 0.5  $\mu m$  by sputtering. For example, this sputtering is performed by using a DC sputtering system and Al as a target while Ar gas is introduced.

Lastly as shown in FIG. 7L, the substrate 40a and portions of the first sacrificial film 44 and low melting point film 42b are etched and removed from the bottom side to expose the gate electrode 41a and first emitter electrode 45 to complete a two-electrode element. For etching Si such as the Si substrate 40a,  $HF+HNO_3+CH_3COOH$  is used, and for etching a silicon oxide film, PSG (low melting point film) or the like,  $HF+NH_4F$  is used.

The effects of the fourth embodiment are similar to those of the first to third embodiments. According to the fourth embodiment, similar to the emitter electrode 45, the gate electrode 41a has a tapered side wall so that a distance between the gate electrode 41a and emitter electrode 45 can be made short. It is therefore possible to raise an electric field intensity at the tip of the emitter electrode and manufacture a field emission element having a low threshold voltage. Also according to the fourth embodiment, the position in height of the emitter electrode 45 is determined by the over-etch depth of the substrate 40 shown in FIG. 7E and the thickness of the first sacrificial film 44 shown in FIG. 7F. A distance between the emitter electrode 45 and gate electrode 41a is determined by the thickness of the first sacrificial film 44. The shape of the emitter electrode 45 and the tapered shape of the gate hole of the gate electrode 41a are determined by the reflow process shown in FIG. 7D and the etching process shown in FIG. 7E. By properly setting these parameters, the position in height of the emitter electrode, the shapes of the gate and emitter electrodes, a distance between the emitter and gate electrodes and the like can be controlled with good reproducibility.

Reflow of the low melting point film of the fourth embodiment will be described more specifically. Other usable low melting point materials include low melting point glass such as PSG, BPSG, BSG, AsSG, AsPSG, and PGSG, frit glass, covar, solder, Si—Ge, or low melting point metal. These materials can be reflowed by baking in a furnace in a

temperature range from 750° C. to 940° C. The reflow temperature depends on an impurity concentration.

It is required that the gate electrode film laminated with a low melting point film and upper and lower layers formed on the gate electrode film have a melting point higher than the reflow temperature. A melting point of polysilicon and amorphous silicon is 1412° C., and the melting points of refractory metals of W and Mo are 3377° C. and 2622° C., respectively. The melting points of refractory silicide films such as  $WSi_2$ ,  $MoSi_2$ ,  $TiSi_2$  and  $TaSi_2$  are 1887° C., 1980° C., 1538° C., and 2200° C., respectively. The melting points of wiring metal materials of Cu, Ag, Au, Rh, Ir, Co and Ni are 1080° C., 960° C., 1063° C., 1966° C., 2450° C., 1495° C. and 1453° C., respectively. These materials have a melting point higher than the reflow temperatures of low melting point film materials such as PSG, BPSG, BSG, AsSG, AsPSG, PGSG, and Si—Ge, and can be used as the materials of films used in the embodiment.

Al or Al alloy used as the gate electrode film material has a melting point of 660° C. which is lower than the reflow temperatures of PSG, BPSG, BSG, AsSG, AsPSG, PGSG, and Si—Ge, and the like. In this case, flowable SOG can be used. For example, FOX (flowable oxide) manufactured by Dow Corning can be used for taper etching low melting point metal such as Al since FOX softens at 200° C. or higher. The low melting point material of this embodiment can therefore be used for a reflow process at a lower temperature.

FIGS. 8A to 8F are cross sectional views of a substrate illustrating the manufacture processes for a field emission element according to the fifth embodiment of the invention. In the embodiment, the manufacture processes for a two-electrode element having an emitter (field emission cathode) and a gate will be described. Also in this embodiment, a tapered shape is formed by reflowing a low melting point film.

Referring to FIG. 8A, a gate electrode film 51 made of first conductive material is formed on a single layer substrate 50 made of, for example, quartz or the like or on a substrate 50 made of a lamination of an Si layer and a silicon oxide film formed thereon. The first conductive material of the gate electrode film 51 is silicon doped with P (phosphorous) or B (boron) and deposited to a thickness of about 0.3  $\mu m$  by low pressure CVD.

For example, the gate electrode film 51 made of silicon is formed under the conditions of a source gas of  $SiH_4$  diluted with He, a substrate temperature of 625° C. and a reaction chamber pressure of 30 Pa. In order to lower the resistance value of the gate electrode film 51, P or B ions are diffused or implanted into the gate electrode film 51.

A low melting point film (low temperature reflow film) 52 is formed on the gate electrode film 51. For example, the low melting point film 52 is made of PSG deposited to a thickness of about 0.5  $\mu m$ . Instead of PSG, other materials such as BPSG, BSG, AsSG, AsPSG, PGSG and Si—Ge may be used.

Next, photoresist material is coated on the low melting point film 52 and etched through photolithography to form a resist pattern 53 having an opening 53a. The low melting point film 52 is isotropically etched via the opening 53a to some extent. In this case, an opening 53b in the low melting point film 52 expands in a lateral direction by side etching. Next, the low melting point film 52 is anisotropically etched in a vertical direction to expose the partial surface of the gate electrode film 51.

Next, as shown in FIG. 8B, the resist mask 53 is removed. By using a process similar to that shown in FIG. 7D of the

fourth embodiment, the low melting point film 52 is heated and reflowed to form a gentle tapered shape as shown in FIG. 8C. Since the low melting point film 52 shown in FIG. 8B has the opening 53b, a low melting point film 52a having a tapered opening 53c can be formed easily.

Next, by using the reflowed low melting point film pattern 52a as a mask, the gate electrode film 51 made of the first conductive material and the low melting point film 52a (changed to a film 52b) are etched to form a recess (gate hole) 52c having a gentle tapered side wall, as shown in FIG. 8D. This etching is preferably an over-etch to etch the substrate 50 by about 0.1  $\mu m$  in depth from the surface of the substrate 50. The depth of this over-etch influences the length and height of an emitter electrode to be later formed.

The diameter of the recess 52c of the gate electrode film 51a is about 0.5  $\mu m$  at the bottom and about 0.7  $\mu m$  at the upper level, and the depth is about 0.3  $\mu m$ .

For example, this etching is performed by using a magnetron RIE system under the conditions of an etching gas of  $CO_2+CHF_3+Ar$  and a reaction chamber pressure of 125 mTorr. Etching rates of the gate electrode film 51 and the low melting point film pattern 52a are 1.2  $\mu m/min$  and 0.9  $\mu m/min$ , respectively.

Next, as shown in FIG. 8E, a first sacrificial film 54 (insulating film) of silicon oxide is isotropically deposited on the whole substrate surface to a thickness of 0.3  $\mu m$  by atmospheric pressure CVD. For example, the first sacrificial film 54 is formed under the conditions of a source gas of  $O_3$  and TEOS and a substrate temperature of 400° C. Under these conditions, the first sacrificial film 54 is deposited inheriting (conformal to) the side wall surface shape of the recess 52c.

Next, a first emitter electrode film 55 of second conductive material such as  $TiN_x$  is isotropically deposited on the first sacrificial film 54 to a thickness of 0.05  $\mu m$  by reactive sputtering. This reactive sputtering is performed by using a DC sputtering system and Ti as a target while a gas of  $N_2+Ar$  is introduced. The first emitter electrode film 55 is therefore formed inheriting (conformal to) the surface shape of the first sacrificial film 54.

Next, by using processes similar to those of the fourth embodiment shown in FIGS. 7H to 7K, a second emitter electrode film 56 made of third conductive material is deposited and etched back to leave a blanket film 56a, and a resistor layer 57 of silicon is deposited to a thickness of about 0.2  $\mu m$  on the first emitter electrode 55 and blanket film 56a by sputtering. An emitter wiring layer 58 made of fourth conductive material such as Al is deposited on the resistor layer 57 to a thickness of about 0.5  $\mu m$  by sputtering.

Lastly, by using a process similar to that of the fourth embodiment shown in FIG. 7L, the substrate 50a and portions of the first sacrificial film 54 and low melting point film 52b are etched and removed from the bottom side to expose the gate electrode 51a and first emitter electrode 55 to complete a two-electrode element, as shown in FIG. 8F.

FIGS. 9A to 9C illustrate methods of reinforcing the emitter electrode with a support substrate according to a modification of the fourth embodiment.

With the method shown in FIG. 9A, a recess on the surface of the emitter electrode 45 of the element subjected to the processes shown in FIGS. 7A to 7G of the fourth embodiment is filled with a planarizing layer 49a made of, for example, spin-on-glass (SOG). Thereafter, the surface of the planarizing film 49a is planarized by chemical mechanical polishing (CMP). Then, a support substrate 49b is adhered to the planarizing film 49a by electrostatic adhesion or by using adhesive.

Thereafter, by using a process similar to that shown in FIG. 7L, the unnecessary portions such as substrate 40a are etched and removed to expose the gate electrode 41a and emitter electrode 45 as shown in FIG. 9A and complete a two-electrode element.

Also with the method shown in FIG. 9B, the emitter electrode 45 of the element subjected to the processes shown in FIGS. 7A to 7G of the fourth embodiment is adhered to a support substrate 49b by using adhesive 49c such as low melting point glass. Thereafter, the unnecessary portions such as substrate 40a are etched and removed by a process similar to the etching process shown in FIG. 7L, to expose the gate electrode 41a and emitter electrode 45 as shown in FIG. 9B and complete a two-electrode element.

With the method shown in FIG. 9C, a recess on the surface of the emitter electrode 45a of the element subjected to the processes shown in FIGS. 7A to 7G of the fourth embodiment is filled with a planarizing layer 49a made of, for example, SOG. Thereafter, the surface of the planarizing film 49a is planarized by CMP. Then, a support substrate 49b is adhered to the planarizing film 49a and emitter electrode 45a by using adhesive 49c such as low melting point glass.

Thereafter, the unnecessary portions such as substrate 40a are etched and removed by a process similar to the etching process shown in FIG. 7L, to expose the gate electrode 41a and emitter electrode 45 as shown in FIG. 9C and complete a two-electrode element.

FIG. 10 illustrates a method of reinforcing the emitter electrode with a support substrate according to another modification of the fourth embodiment. This method is the same as the method shown in FIG. 9C excepting that BPSG is used as the material of a low melting point film 42h. An etching rate of BPSG is about one fourth of that of SiO<sub>2</sub> made of a gas of O<sub>3</sub> and TEOS. Since the etching rate of the low melting point film 42h made of BPSG is slow, it is possible to prevent the low melting point film 42h from being etched completely, and a short circuit of the gate electrode 41a and emitter electrode 45 from being formed.

FIGS. 11A to 11H are cross sectional views of a substrate illustrating the manufacture processes for a field emission element (three-electrode element) according to the sixth embodiment of the invention. Also in the embodiment, a tapered shape is formed by reflowing a low melting point film.

Referring to FIG. 11A, a substrate 60 is formed by depositing an anode electrode 60b made of first conductive material to a thickness of 0.1  $\mu\text{m}$  by low pressure CVD, on either a single layer substrate 60a made of, for example, glass, quartz or the like or on a substrate 60a made of a lamination of an Si layer and a silicon oxide film formed thereon, and by forming a first sacrificial film (insulating film) 60c made of silicon oxide on the anode electrode film 60b to a thickness of 0.1  $\mu\text{m}$  by atmospheric pressure CVD.

In this case, the first conductive material of the anode electrode 60b is silicon doped with P or B in order to lower the resistance value. The anode electrode 60b is formed under the conditions of a source gas of SiH<sub>4</sub> diluted with He, a substrate temperature of 625° C. and a reaction chamber pressure of 30 Pa. The first sacrificial film 60c is formed under the conditions of a source gas of O<sub>3</sub> and TEOS and a substrate temperature of 400° C.

On the first sacrificial film 60c of the substrate 60 formed as above, a gate electrode film 61 made of second conductive material is formed. The second conductive material of the gate electrode film 61 is made of silicon doped with P (phosphorous) or B (boron) and deposited to a thickness of about 0.3  $\mu\text{m}$  by low pressure CVD. For example, this gate

electrode film 61 made of silicon is formed by low pressure CVD under the conditions of a source gas of SiH<sub>4</sub> diluted with He, a substrate temperature of 625° C. and a reaction chamber pressure of 30 Pa. In order to lower the resistance value of the gate electrode film 61, P or B ions are diffused or implanted into the gate electrode film 61.

A low melting point film (low temperature reflow film) 62 is formed on the gate electrode film 61. For example, the low melting point film 62 is made of PSG deposited to a thickness of about 0.5  $\mu\text{m}$ . Instead of PSG, other materials such as BPSG, BSG, AsSG, AsPSG, PGSG and Si—Ge may be used.

Next, by using a process similar to that of the fourth embodiment shown in FIG. 7B, photoresist material is coated on the low melting point film 62 and etched through photolithography to form a resist pattern 63 having an opening 63a about 0.41  $\mu\text{m}$  in diameter at its surface level.

By using the resist pattern 63 as a mask, the low melting point film 62 is isotropically etched to form an opening 62b having a vertical or generally vertical side wall reaching the gate electrode film 61, as shown in FIG. 11B. For example, this etching is performed by using a magnetron RIE under the conditions of an etching gas of CHF<sub>3</sub>+CO<sub>2</sub>+Ar and a reaction chamber pressure of 50 mTorr. In order to prevent the resist from being softened during the etching, it is preferably to cool the bottom surface of the substrate 60 with He.

Next, by using a process similar to that of the fourth embodiment shown in FIG. 7D, the low melting point film 62b is heated and reflowed to form a low melting point film pattern 62d having a tapered recess 62c with a gentle slope upper corner or shoulder.

Next, by using a process similar to that of the fourth embodiment shown in FIG. 7E, the gate electrode film 61 made of the first conductive material and the low melting point pattern 62d are etched to form a recess (gate hole) 62e having a gentle tapered side wall such as shown in FIG. 11D, by using the reflowed low melting point film pattern 62d as a mask. This etching is an over-etch to etch a portion of the first sacrificial film 60c and expose the anode electrode 60b of the substrate 60 and to form a reduced thickness low melting point film pattern 62f. Etching rates of the gate electrode film 61 and the low melting point pattern 62d are about 1.2  $\mu\text{m}/\text{min}$  and 0.9  $\mu\text{m}/\text{min}$ , respectively.

Next, by using a process similar to that of the fourth embodiment shown in FIG. 7F, a second sacrificial film (insulating film) 64 of silicon oxide is isotropically deposited on the whole substrate surface to a thickness of 0.3  $\mu\text{m}$  by atmospheric pressure CVD as shown in FIG. 11E.

Next, by using a process similar to that of the fourth embodiment shown in FIG. 7F, an emitter electrode film 65 of third conductive material such as TiN<sub>x</sub> is isotropically deposited on the second sacrificial film 64 to a thickness of 0.05  $\mu\text{m}$  by reactive sputtering.

Next, a resist mask (not shown) having a predetermined opening is formed on the whole surface of the emitter electrode film 65 by using ordinary photolithography. A portion of the emitter electrode film 65 not used as the cathode is etched and removed through the opening to form a slit opening 66 shown in FIG. 11G. For example, this etching is performed by using a magnetron RIE system under the conditions of a gas of Cl<sub>2</sub> and a reaction chamber pressure of 125 mTorr.

Next, via the slit opening 66, portions of the second and first sacrificial films 64 and 60c are etched to expose the gate electrode 61a, emitter electrode 65a and anode electrode 60b and complete a three-electrode element. For etching the first

and second silicon oxide films and PSG of the low melting point film,  $\text{HF}+\text{NH}_4\text{F}$  is used.

FIG. 12A shows a modification of a three-electrode element of the sixth embodiment. BPSG is used as the material of a low melting point film 62f, instead of PSG. Therefore, during the last process shown in FIG. 11H for etching and removing the unnecessary portions, the low melting point film 62f is hardly removed.

FIG. 12B shows another modification of a three-electrode element of the sixth embodiment. The different structure from the three-electrode element shown in FIG. 12A is that a layer corresponding to the gate electrode layer 61a has a lamination structure of a gate electrode film 61b and an antireflection film 61c such as  $\text{SiN}_x$  and  $\text{SiO}_x\text{N}_y$ , and that the etching rates of first and second sacrificial films 60c and 64a are made generally equal.

Similar to a process shown in FIG. 11G, a resist mask having a predetermined opening is formed on an emitter electrode film 65, and a portion of the emitter electrode 65 not used as the cathode is etched and removed via the opening to form a slit opening 66 such as shown in FIG. 11G. Then, similar to the process shown in FIG. 11H, portions of the second sacrificial film 64a, low melting point film 62f and first sacrificial film 60c are etched and removed via the slit opening 66. In this case, since the etching rates of the first and second sacrificial films 60c and 64a are approximately equal, the unnecessary portions are removed as shown in FIG. 12B to expose the gate electrode 61b, emitter electrode 65a and anode electrode 60b and complete a three-electrode element.

FIG. 14 is a perspective view of a three-electrode element of the third embodiment shown in FIG. 5H. The tip of the emitter electrode 35a is disposed within the gate hole of the gate electrode 31a and has a shape edge like a needle. The three-electrode element has the emitter electrode 35a as a cathode and the anode electrode 30b as a plate. As a predetermined positive potential is applied to the gate electrode 31a, an electron beam is emitted from the emitter electrode 35a toward the anode electrode 30b while being converged.

FIG. 15 is a cross sectional view of a flat panel display using field emission elements of the embodiment described above. Each field emission element used is a two-electrode element formed by the manufacture method of, for example, the first embodiment.

Formed on a support substrate 71 made of insulating material, are a wiring layer 72 made of Al, Cu or the like and a resistor layer 73 made of polysilicon or the like. The wiring layer 72 and resistor layer 73 have predetermined patterns. On the resistor layer 73, a number of gate electrodes 75 having a gate hole (opening) and a number of emitter electrodes 74 whose tips are disposed within the gate holes are disposed to form a field emitter array (FEA). A voltage can be applied independently to each gate electrode 75, although the detailed structure is not shown in FIG. 15. A voltage can also be applied independently to each emitter electrode 74.

Facing an electron source including the emitter electrode 74 and gate electrode 75, an opposing substrate is disposed including a transparent substrate 76 made of glass, quartz, or the like. The opposing substrate has a transparent electrode (anode electrode) 77 made of ITO or the like disposed under the transparent electrode 76 and a fluorescent member 78 disposed under the transparent electrode 77.

The electron source and opposing substrate are joined together via a spacer 80 made of a glass substrate and coated with adhesive, with the distance between the transparent

electrode 77 and emitter electrode 74 being maintained about 0.1 to 5 mm. The adhesive may be low melting point glass.

Instead of the spacer 80 of a glass substrate, a spacer 80 made of adhesive such as epoxy resin with glass beads being dispersed therein may be used.

A getter member 81 is made of Ti, Al, Mg, or the like and prevents emitted gas from attaching again to the surface of the emitter electrode 74.

An air exhaust pipe 79 is coupled to the opposing substrate. By using this air exhaust pipe 79, the inside of the flat display panel is evacuated to about  $10^{-5}$  to  $10^{-9}$  Torr, and then the air exhaust pipe 79 is sealed by using a burner 82 or the like. Thereafter, the anode electrode (transparent electrode) 77, emitter electrode 74, and gate electrode 75 are wired to complete the flat panel display.

The anode electrode (transparent electrode) 77 is always maintained at a positive potential. A display pixel is two-dimensionally selected by an emitter wiring and a gate wiring. Namely, a field emission element at a cross point between the emitter and gate wirings applied with voltages is selected.

The emitter electrode is applied with a negative potential (or ground potential) and the gate electrode is applied with a positive potential, so that electrons are emitted from the emitter electrode toward the anode electrode. When electrons are collided with the fluorescent member 78, light is emitted from the collided area (pixel).

As another embodiment of the invention, the first sacrificial film of the first to sixth embodiments is made of an insulating film such as a silicon oxide film  $\text{SiO}_x$ , a silicon nitride film  $\text{SiN}_x$  and a silicon oxynitride film  $\text{SiO}_x\text{N}_y$ . The first sacrificial film may be made of getter material such as Ti, Ta and zirconium.

The gate electrode and emitter electrode may be made of semiconductor such as polysilicon and amorphous silicon, silicide compound such as  $\text{WSi}_x$ ,  $\text{TiSi}_x$  and  $\text{MoSi}_x$ , or metal such as Al, Cu, W, Mo, Ni, Cr, Hf, and  $\text{TiN}_x$ .

The present invention has been described in connection with the preferred embodiments. The invention is not limited only to the above embodiments. It is apparent that various modifications, improvements, combinations, and the like can be made by those skilled in the art.

What is claimed is:

1. A method of manufacturing a field emission element, comprising the steps of:

- (a) forming a surface layer including a gate film made of a conductive material on a substrate;
  - (b) forming a resist pattern on the surface layer by photolithography, the resist pattern having an opening with a predetermined shape;
  - (c) reflowing the resist pattern to make the opening have an inner diameter gradually reducing toward the substrate;
  - (d) anisotropically etching the gate film by using the reflowed resist pattern as a mask to form an opening through the gate film, the opening having an inner diameter reducing gradually toward the substrate;
  - (e) forming a first sacrificial film covering the gate film having the opening;
  - (f) forming an emitter film made of a conductive material on the first sacrificial film; and
  - (g) removing a portion or a whole of the substrate and a portion of the first sacrificial film to expose the emitter film and the gate film.
2. A method according to claim 1, wherein the surface layer includes only the gate film.

## 21

3. A method according to claim 1, wherein:  
 said step (c) forms the resist pattern having the opening, the opening having the inner diameter gradually reducing toward the substrate, and a cross section of the opening having a gently tapered shape; and  
 said step (d) forms the gate film having the opening, a cross section of the opening having a gently tapered shape.
4. A method according to claim 1, wherein said step (d) anisotropically etches the gate film and the substrate by using the reflowed resist pattern as a mask to form the opening which passes through the gate film and forms a recess in a surface layer of the substrate.
5. A method according to claim 1, further comprising a step of removing the resist pattern after said step (d) and before said step (e).
6. A method according to claim 1, wherein said step (c) reflows the resist pattern by heat treatment.
7. A method according to claim 1, wherein said step (c) performs the heat treatment at a temperature higher than 140° C.
8. A method according to claim 7, wherein said step (c) performs the heat treatment at a temperature higher than 140° C. and lower than 180° C.
9. A method according to claim 6, wherein said step (c) performs the heat treatment at a temperature of 150° C. or higher.
10. A method according to claim 9, wherein said step (c) performs the heat treatment at a temperature range from 150° C. to 160° C.
11. A method according to claim 6, wherein a melting point of the gate film is higher than a temperature of the heat treatment at said step (c).
12. A method according to claim 6, wherein melting points of the substrate and the gate film are higher than a temperature of the heat treatment at said step (c).
13. A method according to claim 1, wherein:  
 the surface layer includes only the gate film;  
 said step (d) anisotropically etches the gate film and the substrate by using the reflowed resist pattern as a mask to form the opening which passes through the gate film and forms a recess in a surface layer of the substrate; and

## 22

- the method further comprises a step of removing the resist pattern after said step (d) and before said step (e).
14. A method according to claim 1, wherein said step (g) etches and removes a portion or a whole of the substrate and a portion of the first sacrificial film.
15. A method according to claim 1, wherein said step (g) etches and removes a whole of the substrate and a portion of the first sacrificial film.
16. A method according to claim 1, wherein:  
 the substrate includes an anode film made of a conductive material and an insulating film formed on the anode film; and  
 said step (g) removes a portion of the first sacrificial film and a portion of the insulating film to expose the emitter film, the gate film and the anode film.
17. A method according to claim 1, wherein the first sacrificial film is made of an insulating material.
18. A method according to claim 1, further comprising a step of filling a recess on a surface of the emitter electrode with a blanket film made of a conductive material, after said step (f) and before said step (g).
19. A method according to claim 1, further comprising a step of adhering the emitter electrode to a support substrate, after said step (f) and before said step (g).
20. A method according to claim 1, wherein:  
 the surface layer has the gate film and a second sacrificial film formed on the gate film;  
 said step (d) forms an opening through the second sacrificial film and the gate film; and  
 said step (e) forms the first sacrificial film covering the surface layer with the opening.
21. A method according to claim 20, wherein the second sacrificial film is an antireflection film.
22. A method according to claim 21, wherein the antireflection film is made of  $\text{SiN}_x$ ,  $\text{SiO}_x\text{N}_y$  or  $\text{TiN}_x$ .
23. A method according to claim 20, wherein the second sacrificial film is made of a getter material.
24. A method according to claim 23, wherein the getter material is Ti, Ta or zirconium.
25. A method according to claim 20, wherein the second sacrificial film is made of an insulating material.

\* \* \* \* \*